

## [54] FUEL FOR ENGINES

[76] Inventor: James Michaels, 26 Valmont Ln., Commack, N.Y. 11725

[22] Filed: Sept. 29, 1972

[21] Appl. No.: 293,576

## Related U.S. Application Data

[63] Continuation-in-part of Ser. No. 150,822, June 7, 1971, abandoned.

[52] U.S. Cl. .... 44/57; 44/58; 44/72; 252/56 R

[51] Int. Cl. .... C10I 1/22

[58] Field of Search .... 44/57, 58, 72; 252/56 R

## [56] References Cited

## UNITED STATES PATENTS

2,497,968 2/1950 Young et al. .... 252/56 R

|           |         |                    |          |
|-----------|---------|--------------------|----------|
| 2,499,984 | 3/1950  | Beavers et al..... | 252/56 R |
| 2,584,803 | 2/1952  | Hannum .....       | 44/72    |
| 2,590,451 | 3/1952  | Perry.....         | 252/56 R |
| 2,611,744 | 9/1952  | Kipp.....          | 252/56 R |
| 2,618,602 | 11/1952 | Bartlett.....      | 252/56 R |
| 2,673,793 | 3/1954  | Brodhacker .....   | 44/53    |

Primary Examiner—Allen B. Curtis

Assistant Examiner—Y. H. Smith

## [57]

## ABSTRACT

Nitroparaffins are added to gasoline together with synthetic lubricants of the ester type (e.g. synthetic jet turbine oil) and are used as fuel in glow engines, jet engines and internal combustion engines in general to improve combustion efficiency, especially by lowering fuel consumption while increasing the output and providing cleaner burning.

16 Claims, No Drawings

## FUEL FOR ENGINES

## CROSS-REFERENCE TO RELATED APPLICATION

This application is a continuation-in-part of my co-pending U.S. application Ser. No. 150,822 filed June 7, 5 1971, now abandoned.

## BACKGROUND OF THE INVENTION

Nitroparaffins, such as mono- and di-nitroderivatives of alkanes having from 1 to 4 carbon atoms, have been 10 proposed for use as fuels to increase engine power in internal combustion engines without attendant penalty of increased engine size or mechanical complexity. Being thermally sensitive, they unfortunately exhibit a tendency to induce pre-ignition when used in internal 15 combustion engines of the reciprocating type. To reduce that tendency, such nitroparaffins are commonly blended with lower alcohols, such as methanol. Previous attempts to blend significant proportions of nitroparaffins into gasoline type engine fuels have failed because these nitroparaffins are not readily miscible in 20 hydrocarbons. For example, nitromethane is only slightly soluble in gasoline, to the extent of no more than about 5 percent. Solubility of nitroparaffins in gasoline can be increased by addition of substantial proportions of aromatic hydrocarbons, such as benzene. This is an expensive expedient and even then the proportions of nitroparaffins which can be incorporated are limited.

The present invention relates to fuels for engines, reciprocating piston engines as well as turbine engines. The invention, in one particular aspect, is concerned with fuel for glow engines used for model aircraft.

It is an object of the present invention to provide fuel for use in internal combustion engines which is better than fuels which are now in use, namely, which provide lower fuel consumption, higher horsepower output and cleaner burning.

Other objects will become apparent from the following description.

## SUMMARY OF THE INVENTION

In accordance with the present invention, it was found that improved fuels for internal combustion engines, viz. reciprocating piston engines, rotary piston engines as well as turbine engines, providing improved combustion efficiency, resulting in lower fuel consumption, increased horsepower output and cleaner burning, are obtained by blending regular petroleum ether, namely gasoline, with certain nitroparaffins, namely nitroalkanes having one or two nitro groups and containing up to four carbon atoms, such as nitromethane, nitroethane, 1-nitropropane, and the like. In accordance with the present invention it was further discovered that these nitroparaffins can be rendered miscible in gasoline by including in the nitroparaffin/gasoline blend a synthetic ester lubricating oil.

Thus, in accordance with the present invention there are provided fuel compositions for internal combustion engines comprising a homogeneous blend of

- A. 5 to 95 parts by volume of gasoline, and correspondingly
- B. 95 to 5 parts by volume of a blend comprising
  - a. 10 to 90 parts by volume of a nitroalkane having one or two nitro groups, and containing up to four carbon atoms, and mixtures thereof, and correspondingly

b. 90 to 10 parts by volume of a normally liquid ester lubricant having a viscosity at 100°F of at least 1 cSt, selected from the group consisting of esters of

- i. linear primary alcohols and linear dicarboxylic acids,
- ii. branched chain primary alcohols and linear dicarboxylic acids,
- iii. branched chain monocarboxylic acids and linear dihydric alcohols and/or polyalkylene glycols,
- iv. linear primary alcohols and branched chain dicarboxylic acids,
- v. neopentyl polyols and monocarboxylic acids, straight chain or branched, and
- vi. mixed complex esters of primary alcohols, straight chain or branched, mono- and dicarboxylic acids, straight chain or branched, and polyalkylene glycols,

and mixtures thereof,

with the proviso that the proportion of ester lubricant in the fuel composition may not exceed 25 percent by volume.

It was unexpected and surprising that addition of even minor proportions of above-described ester lubricant would render perfectly miscible otherwise immiscible nitroalkane/gasoline blends, because neither mineral oil based lubricants nor naturally occurring ester oils, such as castor oil or cottonseed oil are capable of providing such miscibility. Inclusion of ester lubricant in fuel compositions for reciprocating combustion engines has the further advantage of providing internal lubrication within the engine, thereby reducing engine wear and improving engine efficiency. When used in two-cycle engines, particularly air cooled engines, which do not carry their own oil supply as four cycle engines do, the ester lubricant can serve as the normally required lubricant additive, although a separate supply of lubricating oil may be added to the fuel, if desired.

## DETAILED DESCRIPTION OF THE INVENTION

The gasoline component of the present fuel compositions are volatile hydrocarbons having boiling range in the order of 140° to 400°F. Any commercially available type of gasoline is suitable. Usually, such gasolines contain straight chain, branched and cyclic hydrocarbons, in varying proportions, of about 5 to 12 carbon atoms, 45 which may optionally contain minor proportions of aromatic hydrocarbons. They may include natural gasolines, also known as casinghead gasoline, as well as gasoline obtained by cracking of higher boiling hydrocarbons, or by hydrocracking, reformation and alkylation. 50 These gasolines may optionally contain added anti-knock compounds, such as tetraethyl lead, as well as deposit modifiers, antioxidants, metal deactivators, corrosion inhibitors, anti-icing agents, detergents, upper-cylinder lubricants and dyes, such as are usually added to commercial grades of gasoline. However, the straight, unblended hydrocarbons having from about 5 to about 12 carbon atoms, linear as well as branched chain and cyclic, such as n-hexane, n-heptane, n-octane, iso-octane, the various nonanes, decanes and the like are equally suited for use in the present fuel compositions and are intended to be included in the term "gasoline".

Preferred nitroalkanes are the normally liquid nitroalkanes of one to four carbon atoms having one or two nitro groups. They are commercially available. Specific examples of preferred nitroalkanes include nitromethane, nitroethane, 1-nitropropane, 2-nitropropane, 2-nitrobutane as well as 2,2-dinitropropane, although the latter is a solid at normal temperature and pressure. Of these, nitroethane, 1-nitropropane, 2-nitropropane and especially nitromethane are most preferred.

Ester lubricants of the type suitable for use in the fuel compositions of the present invention include those which have found wide use as "synthetic oil" in modern jet engines. These include the commercially available synthetic lubricating oils meeting Military Specifications MIL-L-7808 and MIL-L-9236 of the ester type. Specific examples of commercially available synthetic oils suitable for use in the compositions of the present invention include Texaco SATO No. 7730 Synthetic Aircraft Turbine Oil, Monsanto Skylube No. 450 Jet 20 Engine Oil, and Mobile II Turbine Oil.

Ester lubricants of dicarboxylic acids, straight chain or branched, and primary alcohols, straight chain or branched, generally have the formula



5

10

Mixed complex esters of primary alcohols, straight chain or branched, mono- and di-carboxylic acids, straight chain or branched, and polyalkylene glycols include those having the formulas



and



(V)

wherein

a.  $n$  is an integer of from 2 to 10, preferably from 4 to 8;

b.  $R_1$  and  $R_2$ , which may be the same or different, are alkyl, straight chain or branched, having from 4 to 12 carbon atoms, preferably 6 to 10 carbon atoms.

Preferably, when in formula (I), above,  $-C_nH_{2n}-$  has a straight chain, then  $R_1$  and  $R_2$  are branched, and when  $-C_nH_{2n}-$  is branched, then  $R_1$  and  $R_2$  are straight chain. Straight chain  $R_1$  and  $R_2$  groups are preferred.

Ester lubricants based on dihydric alcohols and/or polyalkylene glycols generally have the formula



35

40

45

50

In above formulas (IV) and (V)  $R_1$ ,  $R_2$ ,  $m$ ,  $n$  and  $r$  have the meanings discussed above in connection with formulas (I) and (II), and  $x$  and  $y$  are integers of from 1 to 4, preferably 1 or 2.

It is to be understood that the above described ester oils may be used in the fuel compositions of my invention in the form of discrete, individual compounds, or as mixtures of isomers, homologues or different compounds. Commercially available ester oils of the above description usually contain additives to improve their performance as lubricants, which additives do not ordinarily adversely affect performance of such oils in my fuel compositions. In general, for reasons of ready availability, use of ester oil in the form of commercially available synthetic ester turbine oils is preferred.

Preferred ester oils, principally for reasons of availability, are those having formula (I), above, derived from dicarboxylic acids. Specific examples of preferred dicarboxylic acids for making ester oils of formula (I) include adipic acid, azelaic acid, and sebacic acid. Specific examples of preferred alcohols for esterification with such acids to make preferred ester oils of formula (I) include straight and, more preferably, branched chain alcohols of 8 to 10 carbon atoms, such as di(2-ethylhexyl) alcohol, oxo-alcohols of 8 to 10 carbon atoms, which are mixtures of isomers and homologues, and 3,5,5-trimethyl hexyl alcohol. Thus, specific examples of preferred ester oils include the adipates, sebacates and azelates of 2-ethylhexyl alcohol, of  $C_8$  to  $C_{10}$  oxo-alcohols, and of 3,5,5-trimethylhexyl alcohol.

A further specific example of a preferred ester oil according to formula (I), above, is the dipelargonate of dipropylene glycol.



60

65

wherein  $R_3$  to  $R_6$ , which may be the same or different, are selected from the group consisting of

a. alkyl, straight chain or branched, having from 1 to 10 carbon atoms, preferably from 1 to 2 carbon atoms, and

b. radicals of the formula



wherein

- i.  $s$  is an integer of from 1 to 4, preferably 1, and
- ii.  $R_7$  has the same meaning as  $R_1$  and  $R_2$  described above in connection with formula (I),

provided that not more than two of the  $R_3$  to  $R_6$  groups may be alkyl groups.

Mixed complex esters of primary alcohols, straight chain or branched, mono- and di-carboxylic acids, straight chain or branched, and polyalkylene glycols include those having the formulas



and



(V)

Ester oils suitable for use in the fuel compositions of the present invention must be normally liquid and must have a viscosity of at least 1 cSt. at 100°F. This minimum viscosity requirement serves as a convenient, practical way of specifying a minimum molecular weight, and thus, carbon atom content requirement for such oils. This designation was chosen in preference over other methods because of its simplicity, because analysis of such oils, especially if in the form of mixtures, is very difficult. Generally, viscosity of these ester oils increases with increasing carbon atom content, i.e. with increasing molecular weight. For example, the sebacinate, azelate and adipate of 2 - ethylhexyl alcohol respectively have viscosities of about 12.5, 11.1 and 8.2 cSt. at 100°F, and of 3.3, 3.0 and 2.4 cSt. respectively at 230°F. Their flashpoints are in the order of 200° to 220°C. While the viscosity limitation is intended as a limitation on lower carbon content, the requirement that these ester oils are "normally liquid" furnishes a limitation on upper level of carbon content, since with increasing carbon contents these esters change from normally liquid oils to greases and waxes.

These ester oils are made by usual procedures involving esterification of the required acid and alcohol in the presence of acidic catalyst, such as sodium hydrogen sulfate, phosphoric acid and its salts, trialkyl or triaryl phosphates, p-toluene sulfonic acid, or mineral acids, under removal of water formed in the reaction by distillation, preferably in the form of its azeotropes with benzene or toluene. Asymmetrical esters and complex esters, of course, require double or multiple step esterification.

For a more complete description of ester oils suitable for use in the fuel compositions of the present invention reference is made to Ullmanns Encyclopaedie der Technischen Chemie, 3rd. Ed., Urban & Schwarzenberg, Muenchen - Berlin (1964), Vol. 15, p. 285 et seq., and references cited therein.

The fuel compositions of the present invention may contain from 5 to 95 percent by volume of gasoline, and from 0.5 to 85.5 percent by volume of nitroalkane. Preferred fuel compositions contain from about 20 to 80 percent by volume, or, more preferably yet, 40 to 80 percent by volume of gasoline, and about 15 to 65 percent, more preferably 15 to 45 percent by volume of nitroalkane.

The ester oil is preferably employed in minimum amount required to provide a homogeneous liquid fuel compositions. Use of less than that amount results in non-homogeneous compositions, with concomitant physical separation of liquid components into layers, and use of excess amounts of ester oil is wasteful and may result in excess carbon deposition within the engine, fouling of sparkplugs and generally unsatisfactory engine operation. No general rule can be set down fixing precise amounts of ester oil required to achieve homogeneity of the compositions, since that amount depends on variables such as the type of gasoline, nitroalkane and ester oil, as well as the proportions in which gasoline and nitroalkane are incorporated into the composition. However, the required amounts of ester oil are readily determined by simple experimentation of routine nature, e.g. by first adding the nitroalkane to the gasoline in desired amount, then adding the ester oil in small portions, followed by thorough mixing after each addition, until a homogeneous blend is obtained. As a general guide, use of ester oil in proportions of

from 1 to 4 parts of ester oil to 8 parts of nitroalkane will ordinarily provide a homogeneous blend.

It has further been found that it is sometimes advantageous to add small amounts of propylene oxide, C<sub>3</sub>H<sub>6</sub>O, to the fuel compositions of the present invention, to obtain further improvement in engine operation.

Also, it is often desirable to use blends of various nitroalkanes. For example, a blend of 3 parts of nitromethane, 1 part nitroethane, 2 parts nitropropane and ½ part propylene oxide was found to be most efficient. Other possible blend compositions may be as follows: 4 parts nitroethane and 1 part nitromethane; 4 parts nitromethane, 3 parts propylene oxide and 1 part nitroethane; 2 parts nitromethane, 1 part nitroethane and 1 part nitropropane; 1 part nitroethane and 1 part nitropropane; 1 part nitromethane, 1 part nitroethane and 1 part nitropropane.

A specific example of a preferred fuel composition for use in glow plug engines comprises: about

80 parts by volume of gasoline,  
16 parts by volume of nitromethane, and  
4 parts by volume of ester lubricant

(e.g. Mobile II Turbine Oil, sold by Mobil Oil Co.)

The fuel mixture can be used in glow engines which will then perform on par with or better than alcohol base fuels containing nitroalkane, such as nitromethane. The advantages of using the fuel of the present invention are found in lower fuel consumption due to high BTU of energy developed resulting in higher horsepower output and cleaner burning, since the added blends (of nitroalkane and their mixtures) improve combustion efficiency. The same advantages occur when this fuel is used in other internal combustion engines or jet engines.

Since various changes and modifications may be made in the invention without departing from the spirit or essential characteristics thereof, it is intended that all matter contained in the above description shall be interpreted as illustrative only, the invention being limited only by the scope of the appended claims.

I claim:

1. Fuel composition for internal combustion engines comprising a homogeneous blend of

A. 5 to 95 volume percent of gasoline, and correspondingly

B. 95 to 5 volume percent of a blend comprising

a. 10 to 90 volume percent of a nitroalkane having one or two nitro groups, and containing up to four carbon atoms, and mixtures thereof, and correspondingly

b. 90 to 10 volume percent of a normally liquid ester lubricant having a viscosity at 100°F. of at least 1 cSt. selected from the group consisting of esters of

i. primary alcohols, linear or branched chain, and dicarboxylic acids, linear or branched chain, having the formula



wherein *n* is an integer of from 2 to 10 and R<sub>1</sub> and

R<sub>2</sub>, which may be the same or different, are alkyl, straight chain or branched, having from 4 to 12 carbon atoms,

ii. monocarboxylic acids and dihydric alcohols and/or polyalkylene glycols having the formula



wherein  $m$  is an integer of from 2 to 12,  $r$  is an integer of from 1 to 10, and  $R_1$  and  $R_2$  have the afore-stated meanings,  
iii. neopentyl polyols and monocarboxylic acids, straight chain or branched, having the formula



wherein  $R_3$  to  $R_6$ , which may be the same or different, are selected from the group consisting of (1) alkyl, straight chain or branched, having from 1 to 10 carbon atoms, and (2) radicals of the formula  $C_sH_{2s}OOCR_7$ , wherein  $s$  is an integer of from 1 to 4, and  $R_7$  is alkyl, straight chain or branched, having from 4 to 12 carbon atoms, with the proviso that not more than two of the  $R_3$  to  $R_6$  groups may be alkyl, and  
iv. mixed complex esters of primary alcohols, straight chain or branched, mono- and dicarboxylic acids, straight chain or branched, and polyalkylene glycols, having the formulas



and



wherein  $R_1$ ,  $R_2$ ,  $m$ ,  $n$ , and  $r$  have the afore-stated meanings and  $x$  and  $y$  are integers of from 1 to 4,

and mixtures thereof,

with the proviso that the proportion of ester lubricant in the fuel

2. Fuel composition according to claim 1 containing from about 20 to 80 percent by volume of gasoline and from about 15 to 65 percent by volume of nitroalkane.

3. Fuel composition according to claim 1 containing from about 40 to 80 percent by volume of gasoline and from about 15 to 45 percent by volume of nitroalkane.

4. Fuel composition according to claim 3 wherein the nitroalkane is nitromethane.

5. Fuel composition according to claim 1 wherein the

40

50

ester lubricant has the formula



wherein

- 5 a.  $n$  is an integer of from 2 to 10, and  
b.  $R_1$  and  $R_2$ , which may be the same or different, are alkyl, straight chain or branched, having from 4 to 12 carbon atoms.

6. Fuel composition according to claim 5 containing from about 20 to 80 percent by volume of gasoline and from about 15 to 65 percent by volume of nitroalkane.

7. Fuel composition according to claim 5 containing from about 40 to 80 percent by volume of gasoline and from about 15 to 45 percent by volume of nitroalkane.

8. Fuel composition according to claim 7 wherein the nitroalkane is nitromethane.

9. Fuel composition according to claim 1 wherein the ester lubricant has the formula



wherein

- 20 a.  $m$  is an integer of 2 to 12,  
b.  $r$  is an integer of 1 to 10, and  
c.  $R_1$  and  $R_2$ , which may be the same or different, are alkyl, straight chain or branched, having from 4 to 12 carbon atoms.

10. Fuel composition according to claim 9 containing from about 20 to 80 percent by volume of gasoline and from about 15 to 65 percent by volume of nitroalkane.

11. Fuel composition according to claim 9 containing from about 40 to 80 percent by volume of gasoline and from about 15 to 45 percent by volume of nitroalkane.

12. Fuel composition according to claim 7 wherein the nitroalkane is nitromethane.

13. Fuel composition according to claim 1 containing about 80 parts by volume of gasoline, about 16 parts by volume of nitromethane, and about 4 parts by volume of ester lubricant.

14. Fuel composition according to claim 13 wherein the ester lubricant is an ester of branched chain primary alcohol and linear dicarboxylic acid.

15. The method of creating energy which comprises burning a fuel according to claim 1 in an internal combustion engine.

16. The method of creating energy which comprises burning a fuel according to claim 14 in a glow plug engine.

\* \* \* \* \*

55

60

65

UNITED STATES PATENT AND TRADEMARK OFFICE  
CERTIFICATE OF CORRECTION

PATENT NO. : 3,900,297  
DATED : August 19, 1975  
INVENTOR(S) : James Michaels

It is certified that error appears in the above-identified patent and that said Letters Patent are hereby corrected as shown below:

Column 3, line 15, delete "metting" and substitute therefor  
--meeting--.

Column 7, line 40 (last line of claim 1), add --composition  
may not exceed 25 percent by volume.--.

Signed and Sealed this  
twenty-fifth Day of November 1975

[SEAL]

Attest:

**RUTH C. MASON**  
*Attesting Officer*

**C. MARSHALL DANN**  
*Commissioner of Patents and Trademarks*